

March 13, 1928.

1,662,676

W. C. JAMES

OUTDOOR SIGN

Filed Oct. 29, 1923



INVENTOR:

Will C. James

BY

Albert Allen  
ATTORNEYS.

Patented Mar. 13, 1928.

1,662,676

# UNITED STATES PATENT OFFICE.

WILL C. JAMES, OF NORWOOD, OHIO, ASSIGNOR TO THE KEMPER-THOMAS COMPANY, OF NORWOOD, OHIO, A CORPORATION OF OHIO.

## OUTDOOR SIGN.

Application filed October 29, 1923. Serial No. 671,406.

My invention relates to an outdoor sign formed of fibreboard, as distinguished from metal signs generally. For many years I have been engaged in the manufacture of 5 outdoor signs for advertising purposes to the extent to make certain that a properly treated piece of fibreboard will outlast, for the desired life of a sign, any ordinary metal sign of a character within range of economy.

10 The processing of such outdoor signs of fibreboard is, however, a matter of great importance in assuring a long life, maintenance of brilliancy of coloring and assurance of perfect application of printing inks and 15 colors.

It is my object in this invention to provide a process of preparing outdoor signs of fibreboard so as to fill and cap all pores with a moisture resistant material, to prepare 20 a satisfactory printing mat or surface upon the board, to print or decorate the board and finally to coat the printed surface together with the board with a varnish-like material, and to protect the edges of the 25 board.

While I speak in the specifications that follow of a piece of fibreboard, it should be understood that what I refer to is a piece of material having fibreboard on the outside, 30 without reference to the number of plies of fibrous material, or the presence or absence of a stiffener or filler of any other nature.

I am aware that signs have been manufactured of cardboard for many years, in which attempts have been made to render the sign 35 waterproof, but never, so far as I am aware, with complete success, and my present invention represents the refinement in processing 40 devised by me, whereby the boards have been produced in a way which almost entirely precludes the entrance of moisture into the board, and the consequent disintegration of the paper or scaling off of the printed 45 matter, as is frequently the case with other signs.

I accomplish my objects by the certain process to be hereinafter more specifically pointed out and claimed.

50 In the drawing:

Figure 1 is a perspective view of one of my signs.

Figure 2 is a cross section thereof.

The fibreboard either after being cut to 55 size or in the large mill size sheets is, if

necessary, put through a process to remove a percentage of the moisture. It is not so important that any one given percent of moisture should remain in the board, but rather that the sheets before treatment 60 should be brought to a uniform, fairly low moisture content, so that a regular system of impregnating can be followed without resulting in an irregular product. The resultant board is now immersed in a bath of 65 either hot or cold compound suitable for impregnating it, the temperature in no case being greater than about 200° F., since much higher temperatures tend to disintegrate the paper. The impregnating material may 70 consist of oils, fats, protein solutions, or mixtures thereof—in fact, the primary qualification is that the mass shall be water-insoluble and possess the necessary qualities of adhering firmly to the paper fibre and a setting power or melting point sufficiently high 75 to prevent its being melted by the heat of the sun. Immersion of the board in hot molten waxes such as ceresin, ozokerite, carnauba or sandarac, or mixtures thereof may be suitable 80 for the purpose. In my preferred process, I employ a solution of casein and the resultant impregnated board is thereafter treated with formaldehyde, said two substances combining with each other so as to 85 form an almost ideal medium.

After thorough impregnation of the board and practically complete filling of the spaces between the fibers, the board is run 90 between rollers under light pressure to remove the excess from the surface. The resulting thoroughly impregnated board is now white or color coated with a combination consisting of a drying varnish and a pigment and may then be dried, and subsequently 95 printed, stenciled or lithographed in as many colors as may seem desirable for working out the design or announcement. The printed board is now varnished with one or more coats of long-lived, moisture resisting varnish to render the board as nearly weatherproof as possible. It is then bound with metal strips crimped around its edges to stiffen it, and also to exclude moisture getting in between the plies, where this is a 100 danger, due to the way the board is built up.

The attached drawing shows the ideas graphically both flat and cross section, corresponding numerals indicating the different parts. 1 is the board, 2 the first coating, 110

3 the second coating and 4 the varnish coating. The binding 5 is then applied as shown.

The particular point which I wish to 5 cover is the method of impregnating thoroughly the fibreboard to be used with an inexpensive water-insoluble filling material, and the use of such filled fibreboard in combination with the other products to form a 10 sign. Such a combination will have very long life and will render advertising in such a manner less expensive.

Having thus described my invention, what I claim as new and desire to secure by Letters Patent, is:

1. The process of manufacturing an outdoor sign, consisting first in filling the interstices of a fiber board sheet, by capping them with an insolubilized casein, secondly coating the board with an ink receptive medium, 20 thirdly decorating the sign with a suitable announcement, fourthly varnishing the board.

2. The process of manufacturing an outdoor sign consisting first in filling the interstices of a fiber board sheet by capping them with an insolubilized colloid, secondly coating the board with an ink receptive medium of a type which will receive a decoration im-

printed thereon, thirdly decorating the sign 30 with a suitable announcement printed over the coating of the second step and fourthly varnishing the board.

3. The process of manufacturing an outdoor sign consisting of treating a fibre board with a casein solution and formaldehyde as a coagulant, color coating the resulting board with a pigment in a drying oil, printing an announcement thereon, and varnishing the surface front and back.

4. The process of manufacturing an outdoor sign which includes the steps of capping the pores of a fibre board sheet to prevent penetration of moisture, varnish, and ink by treatment with a casein solution and formaldehyde, color coating the board, and printing an announcement upon the resulting board, and varnishing the resulting sign, face and back.

5. The process of producing a fibre board sign by filling and capping the pores on the surface of a fibre board by means of an insolubilized protein solution, forming an announcement upon the board so treated, and applying a transparent coating of weather- 55 proof nature over the board.

WILL C. JAMES.